

Jan. 22, 1935.

F. G. BAENDER

1,988,773

## RECLAIMING USED LUBRICATING OILS

Filed April 11, 1932



## UNITED STATES PATENT OFFICE

1,988,773

## RECLAIMING USED LUBRICATING OILS

Frederick G. Baender, Corvallis, Oreg.

Application April 11, 1932, Serial No. 604,493

2 Claims. (Cl. 196—16)

My invention relates to the reclaiming of lubricating oils after use in internal combustion engines.

It is well known that lubricating oil used in internal combustion engines requires to be changed at the end of definite periods, not because of the destruction of its lubricating properties, but because it has accumulated so much foreign matter and become mixed with water and gasoline, or other light petroleum components to such extent that its further use is apt to be injurious to the moving parts of the engine.

Various attempts have been made to devise a method suitable for reclaiming such oil, but the oil so reclaimed has not as a general rule been favorably received by the public, largely due to the fact that its color is deterring, being so dark as compared with fresh, standard lubricating oil, as to make an unfavorable impression and induce hesitancy on the part of the public to use the reclaimed oil. In fact, such reclaimed oil has a greater lubricating value than unused oil, for the reason that the unsaturated hydrocarbons of the unused oil are broken down and driven off by the action of the engine on the oil, and the foreign particles it may originally contain are separated, so that they may be removed during the reclaiming method.

Difficulty has also been experienced in removing the gasoline and other light hydrocarbons and water from the lubricating oil without at the same time "cracking" or volatilizing the lighter components of the lubricating oil and destroying or reducing its value as a lubricant.

The object of my invention is to provide a method for reclaiming and purifying used lubricating oils without wastage, and for restoring its original color.

My invention also provides a method by which, by proper control of the temperature and pressure a larger percentage of the higher or more volatile components of the oil may be separated from the oil being treated, by which to produce, if desired, a heavier body in the lubricating oil than it originally had.

With my invention also the vapors and gases driven off from the oil may be condensed and saved for further treatment, preventing their escape to the atmosphere, which is undesirable because of their disagreeable odor.

My invention provides a practical and economical apparatus adapted to carry out my process. I attain my above objects in a method which comprises first sludging the used lubricating oil to induce the precipitation of its foreign matter,

neutralizing the body of oil, then removing the neutralizing agent and intermixing fuller's earth or other earthy substance with the body of oil, heating the resultant commixture under constant stirring in a closed retort under pressure to a temperature of approximately 350 degrees F. to convert the moisture in the oil into steam, then permitting such steam to escape gradually so as to prevent carrying off of oil particles with the steam, continuing the heating but raising the temperature to approximately 450 degrees F. to distill off the volatile components of the oil not to be retained, injecting small portions of water into the heated oil which flash into steam and carry off the suspended fine particles of foreign matter from the oil, cooling the oil before exposing it to the air, and filtering the oil to remove the fuller's earth.

My method and apparatus provided therefor are hereinafter described in detail with reference to the accompanying drawing.

In the drawing:

Fig. 1 shows a preferred form of my apparatus I employ for carrying out my method of reclaiming used lubricating oil; and

Fig. 2 shows the details of construction of the collapsible mechanical stirrer I provide, removed from the retort.

Referring now to the drawing: My apparatus comprises an open vessel or tank 1, provided with a funnel-like bottom 2 having a valve controlled outlet 3 and provided with a pipe 4 leading from a source of compressed air, not shown, which discharges into the bottom of the said tank, for agitating the oil placed therein.

A pipe 5 is connected to the tank 1, above the funnel-like bottom 2 and to an inlet 6 in the top of a cylindrical retort 8, the said retort 8 preferably being arranged on a lower level than the tank 1, so that the oil may flow into the retort by gravity.

The said inlet 6 is controlled by a valve 9. The retort is also provided at the top with a relatively small outlet 10 for the gases and vapors and is controlled by a valve 11 and connected to a pipe 12 leading to a condenser 13.

An outlet 14 controlled by a valve 15 is provided in the bottom of the retort 8 connected by a pipe 16 with a set of cooling coils 17 which are in turn connected thru a pipe 18 with a filter 19, comprising a closed tank in which is located a series of bag-like filter elements 20 connected with an outlet pipe 21. The oil passes from the tank 19 to the interior of the filter elements 20 and then out thru the outlet pipe 21 and is thus

separated from any solid material that may be contained in it. The filter elements 19 are constructed of suitable fabric material and are provided with relatively stiff wire framework 22, 5 adapted to hold them distended, as illustrated in the figures. By providing this type of filter, the filter elements 20 may be lifted out of the tank 19, as a unit, and readily cleaned, since the filtered material will collect on the outside.

10 The retort 8 is provided with electrical heating elements 25 and with a mechanical stirrer mounted on a horizontally arranged shaft 27 which extends thru one end wall of the retort and is provided with a driven pulley 28.

15 The stirrer 26 is connected by pivoted links 29 to arms carried by the shaft 27, so that it may be collapsed as illustrated in Fig. 2 and inserted thru a relatively small hole 31 in the end of the retort. The hole 31 is closed by a plate 32 in which one 20 end of the shaft 27 is journaled. Thus the stirrer may be inserted and removed without dismantling the retort and the centrifugal force of its rotation will hold it extended as illustrated in Fig. 1.

25 A spray pipe 35 connected with a source of cold water is provided in the bottom of the retort 8.

In carrying out my method, the used lubricating oil to be reclaimed is placed in the open vessel or tank 1 and an acid such as sulphuric acid 30 is introduced to cause the precipitation of the heavier foreign matter present in the oil.

The amount of sulphuric acid added will depend on the character of the oil and the amount of foreign matter present and may be determined 35 by the appearance and "feel" of the oil.

I then agitate the oil and acid by means of compressed air introduced into the bottom of the tank thru the pipe 4 to insure a thorough intermixture of the oil and acid. The oil is then allowed to stand to permit the precipitants to settle to the bottom in the form of sludge which 40 may be drained off and wasted thru the outlet 3.

After draining off the sludge I introduce a sufficient quantity of a base, such as lime, to neutralize the acid and again agitate and then drain off and waste the resulting precipitants. Of course, should the used oil being treated contain 45 very little or no foreign matter this step may be omitted.

After the lime precipitants are drained off, I add a quantity of fuller's earth or other earthy material, approximately one-half to three-fourths pounds to the gallon and allow the resulting commixture to flow by gravity into the retort 8 thru the pipe 5. The commixture is then thoroughly intermixed by the stirrer 26 which is maintained in continuous operation to prevent the fuller's earth from settling to the bottom of the retort. 55

60 The valves 9 and 11 are then closed and the heating elements 25 are actuated to heat the commixture to a temperature of approximately 350 degrees F., under a resulting pressure of about 40 pounds to the square inch, which drives out 65 the water content both free and emulsified.

As soon as the water content is driven out of the oil, which requires approximately one hour, depending upon the character of the oil being reclaimed, I open the valve 11 controlling the 70 outlet 10 and permit the steam to escape slowly thru the pipe 12 to the condenser 13, where it is condensed and wasted, but is prevented from escaping to the atmosphere, the latter being undesirable because of its disagreeable odor.

75 Further by driving off the water content of the

commixture in a closed retort, loss of oil, which would be carried off by the escaping steam is prevented and by then releasing the steam and allowing the pressure to fall gradually to atmospheric, the escaping steam cannot carry any of the oil with it. 5

It is to be noted that by carrying on the heating of the oil to drive off the water content, in a closed retort, I materially lessen the time required, for otherwise the heating of the oil at 10 this temperature would cause it to boil over, and be ejected from the retort. In fact at a temperature of 350 degrees F. in an open retort, the oil would all be ejected within a relatively short time, approximately five minutes. 15

Further, the gradual fall of pressure permits a further gradual vaporization of the water content of the commixture, prevented by the initial higher pressure and thus violent boiling or ebullition is prevented which would also tend to eject 20 a portion of the oil from the retort.

The heating of the commixture is then continued at a temperature of approximately 450 degrees F. to volatilize and drive off the hydrocarbon components which comprise the gasoline 25 and other more volatile hydrocarbons intermixed with the oil.

It is to be noted that during this step, I may, if desirable, raise the temperature of the commixture sufficiently to volatilize and drive off a larger 30 percentage of the lighter components of the lubricating oil to produce a lubricating oil having a heavier body.

The escaping gases from the commixture which are condensed in the condenser 13 may either be 35 wasted or saved for further treatment to separate the gasoline components from water and other undesirable components. However, it is essential that they be condensed and not allowed to escape to the atmosphere because of the explosive properties particularly at high temperature. 40

After the said volatile components of the commixtures are driven off, I introduce a small quantity of cold water thru a spray pipe 30 located in the bottom of the retort, which is immediately 45 flashed into steam by the heat of the commixture and carries off the remaining more volatile components, foreign matter and other impurities and clarifies and deodorizes the oil.

By introducing cold water into the commixture, 50 which immediately flashes into steam, the volume of the water increases approximately 1200 times and thus produces an explosive effect, which breaks away the remaining solid particles intimately intermixed with the oil, which are carried 55 away by the steam as it passes upwardly thru the oil.

Finally, as the last step of my method, I open the valve 15 controlling the outlet 14 and discharge the commixture thru the pipe 16, to the 60 cooling coils 17 and to the filter 19 where the fuller's earth and other remaining solid particles are removed. Such cooling of the commixture is essential, for otherwise at a temperature above 450 degrees F. the oil would tend to flash into 65 combustion on exposure to the atmosphere and in any event will become oxidized and turn black, which is of course to be avoided.

Further, in order to avoid using a pump to draw the commixture from the retort 8 and force 70 it thru the filter 19, I close the valve 11 at the end of the heating period and continue to inject water, which, turning to steam, creates a pressure in the retort and forces the commixture from the retort and thru the filter without auxiliary means. 75

By using steam for this purpose, I provide a gas, which does not react with the oil. To use air for this purpose would oxidize the oil and cause it to turn black which, as mentioned, is undesirable.

Finally when the retort 8 is completely empty, the steam tends to pass thru the cooling coils 17 and be condensed to water which would intermix with the oil, but the temperature of the oil in passing thru the said cooling coils is only lowered to approximately 220 degrees F. and thus the intermixed water immediately turns to steam and passes off in the form of vapor.

I claim:

1. The herein described method of reclaiming used lubricating oil comprising mechanically agitating the oil and heating the oil under pressure in a closed retort to a temperature of approximately 350° F., to effect removal of water from the oil by vaporization and to restrain ebullition and the carrying off of particles of oil with the water vapor; then opening the retort and permitting the generated steam to escape gradually until pressure within the retort is reduced to atmospheric; then further heating the oil with the retort open to approximately 450° F. to drive off the more volatile components of the oil and discharging

these components from the retort thru a cooling coil; then, while maintaining the last mentioned temperature, clarifying and deodorizing the oil by introducing into the bottom thereof small jets of cold water whereby to cause flashes of steam to surge thru the oil, then withdrawing the oil from the retort thru a cooling coil without exposure to the atmosphere, and finally filtering it.

2. In the reclaiming of used lubricating oil the herein described steps comprising first dehydrating the oil by heating the oil under pressure in a closed retort to a temperature of approximately 350° F., to effect removal of water from the oil by vaporization and to restrain ebullition and the carrying off of particles of oil with the water vapor; then opening the retort and permitting the generated steam to escape gradually until pressure within the retort is reduced to atmospheric; then further heating the oil with the retort open to approximately 450° F. to drive off the more volatile components of the oil, then, while maintaining the last mentioned temperature, clarifying and deodorizing the oil by introducing into the bottom thereof small jets of cold water whereby to cause flashes of steam to surge thru the oil.

FREDERICK G. BAENDER.